

## UNITED STATES PATENT OFFICE.

PORTER H. BRACE, OF PITTSBURGH, PENNSYLVANIA, ASSIGNOR TO WESTINGHOUSE ELECTRIC & MANUFACTURING COMPANY, A CORPORATION OF PENNSYLVANIA.

## ALLOY OF TANTALUM.

No Drawing.

Application filed April 18, 1919. Serial No. 291,033.

My invention relates to alloys and it has, for its primary object, the provision of alloys which shall be highly resistant to acids, strong, reasonably ductile and resistant to 5 oxidation.

Another object of my invention is to provide alloys, possessing the foregoing characteristics, which shall be relatively hard so that they may be employed, not only in 10 the formation of acid-proof ware, but also in the manufacture of cutting tools.

A still further object of my invention resides in the formation of alloys, of the character described, which may be satisfactorily 15 utilized in the manufacture of electrical-resistance elements.

More particularly, my invention relates to alloys comprising, as one ingredient, tantalum or a metal of the tantalum group, 20 such as columbium or niobium, together with nickel or another metal of the nickel group, such as cobalt, with, the addition of a metal of the chromium group, preferably chromium.

I have found that alloys of this character are substantially white in color; take a fine 25 polish and may be worked by the usual methods, such as forging, rolling and drawing. Such alloys are also highly resistant 30 to acids, resistant to oxidization, and possess, in many instances, such degree of hardness that they may be utilized in the manufacture of cutting tools.

While the members of the tantalum group 35 are, for my purposes, substantial equivalents, I prefer to employ tantalum and I have found that alloys of tantalum and nickel or of tantalum and cobalt, possess great strength and considerable ductility 40 and are highly resistant to acids. As a rule, I prefer to employ at least 25% tantalum and from 1% to 75% nickel or cobalt, the two being interchangeable. An alloy of 45 this character is highly resistant to acids and may, therefore, be utilized in the manufacture of acid-proof ware.

I employ as a hardener, in connection with the tantalum and nickel alloy, a certain proportion of any of the metals of the chro-

mium group. For instance, an alloy highly 50 resistant to acids and also resistant to oxidization may comprise from 5% to 30% chromium, together with tantalum and nickel in the proportions of 75% nickel to 25% tantalum. In place of the chromium, 55 I may substitute molybdenum or tungsten which will harden the alloy materially, rendering it particularly adaptable for the manufacture of cutting tools. The alloys containing a metal of the tantalum group 60 are also suitable for the manufacture of electrical-resistance elements.

An alloy embodying my invention may be formed by any of various well known methods as, for example, by mixing the metals in a powdered form, compressing them at relatively high pressure and applying a relatively high heat in a crucible previously disposed in a vacuum. The above mentioned method is set forth in the Journal of the 70 Iron and Steel Institute on pages 390 and 391, No. 1, 1916. The alloy may also be readily produced by the reduction of mixed oxides of the metals as, for example, by the well known alumino-thermic methods or by 75 reducing mixed oxides of the metals employed, to form carbides, and by subsequently melting the carbides, thus formed, in a vacuo, as described in a copending application filed by me Apr. 18, 1919, Serial 80 No. 291,034, and assigned to the Westinghouse Electric & Manufacturing Company.

While nickel and cobalt are substantial 85 equivalents, in alloys of this character, I find that the substitution of cobalt for nickel results in alloys which, in general, are harder but somewhat less resistant to acid attacks. Their ductility is also somewhat less.

Addition of chromium or a metal of the 90 chromium group to alloys of tantalum and nickel or tantalum and cobalt greatly increases the resistance of the alloys to oxidization and also, in general, increases their hardness and resistance to acid attack.

In view of the large number of closely 95 related alloys comprehended by my invention and because of the numerous uses to

which they may be put, it will be appreciated that my invention is to be limited only as indicated in the appended claim.

I claim as my invention:

An alloy resistant to acids and oxidation comprising 5 to 30% chromium and the remainder tantalum and nickel in substantially the proportions of 1 to 75% nickel and 25 to 99% tantalum.

In testimony whereof, I have hereunto 10  
subscribed my name this 3rd day of April,  
1919.

PORTER H. BRACE.